

Jan. 16, 1940.

P. GORLICH

2,187,234

PROCESS OF PRODUCING A PHOTOELECTRIC TUBE

Filed Feb. 25, 1938



Inventor  
Paul Gorlich  
By Binger and  
S. Stern, atty.

## UNITED STATES PATENT OFFICE

2,187,234

61

PROCESS OF PRODUCING A PHOTOLEC-  
TRIC TUBEPaul Görlich, Dresden, Germany, assignor to  
Zeiss Ikon Aktiengesellschaft, Dresden, GermanyApplication February 25, 1938, Serial No. 192,628  
In Germany February 25, 1937

1 Claim. (Cl. 250—27.5)

The invention relates to a method of producing a photoelectric tube.

It is an object of the invention to produce a photoelectric tube requiring only small quantities of photoelectric substances to attain a high degree of sensitiveness.

Another object of the invention is to produce a photoelectric tube of high sensitiveness in a simple manner and to effect the regulation of the proportions of materials required automatically during the method.

It is furthermore, an object of the invention to regulate the sensitiveness of the tube during its production in accordance with the compound from which the deposits in the tube are released in predetermined quantity.

With these and other objects in view, the invention is described in the following specification with reference to the accompanying drawing.

20 The drawing illustrates diagrammatically a device which may be employed for practicing the method of the present invention.

In producing a photoelectric tube, according to the present method, the vessel or bulb of the tube is first produced in customary manner and its inner wall is coated in any desired known way with a metal, as for instance, silver or copper.

The improvement of the present method of completing the production of this tube, includes

30 the step of depositing by vaporization an alkali metal in the form of a thin layer upon the inner metal coating of the tube. For this purpose a tubular reservoir connected with the bulb of the tube may contain a predetermined quantity of a

35 compound of the alkali metal, or a compound of alkali metal may be disposed upon a carrier within the tube itself. Upon applying heat to the compound of alkali metal, the alkali metal itself is liberated from the compound in predetermined amounts. This step, therefore, will result in the deposit, and regulation of the deposit, of a

40 condensed layer of alkali metal on the metal coating in the tube.

When it is desired to leave certain areas in the interior of the tube free of this deposit of alkali metal, the respective areas of the tube may be heated to a temperature preventing the condensation of the vapor of alkali metal on the respective areas.

50 The method of the invention includes, furthermore, the step of converting the deposited alkali metal into an oxide without necessarily effecting the oxidation of other metallic deposits in the tube. For this purpose a predetermined amount of oxygen may be introduced into the tube, or may

be generated within the tube itself. In the first named case, the bulb may be connected with another tubular reservoir within which a compound adapted to release oxygen is disposed. Upon heating this compound, as for instance, by applying heat to the reservoir a predetermined quantity of oxygen will be liberated and this quantity is just sufficient to convert the layer of alkali metal into a photoelectrically active oxide of alkali metal. Preferably caesium is used as alkali metal which in this described manner is converted into caesium oxide.

55 After this oxide layer has been produced free alkali metal is deposited by vaporization upon the oxide. This free alkali metal may be supplied from another reservoir connected with the bulb of the tube or may be supplied in other suitable manner. The reservoir containing free alkali metal is heated to cause the alkali metal to be vaporized in which condition it passes into the bulb of the tube to be deposited therein as a condensate upon the previously produced oxide layer.

60 The vaporization of the free alkali metal to constitute a top layer on the deposit of the oxide of alkali metal is continued until a test shows that the maximum sensitiveness of the tube has been attained.

65 As a simple test the tube may be energized by light, during this last step of depositing the free alkali metal, and the electric current produced by the tube measured by a galvanometer. As soon as the galvanometer indicates a maximum current, the deposition of free alkali metal is terminated.

70 In the drawing the bulb 1 of the photoelectric tube is connected to the high-vacuum-pump 5 by means of a pipe line 2, 3, and 4. Before starting the high-vacuum-pump a so called initial or rough vacuum is produced in the bulb 1 by connecting the pipe line to a rough-vacuum-pump (not shown). Then, before starting the electrically heated high-vacuum-pump 5 the cocks 7 and 8 must be closed. After starting the high-vacuum-pump the cock 9 is opened and the bulb 1 is exhausted to an extremely high vacuum. Then the reservoir 10, containing a photoelectrically active metal e. g. caesium, is heated by means of a gas burner or electrically in any known manner. The caesium evaporates and passes over the branch line 11 into the bulb 1. The heating may also be effected in such manner, that only a portion of the caesium in the reservoir is vaporized and passed into the bulb 1. After opening the cock 12 the reservoir 13, containing a substance

10

15

20

25

30

35

40

45

50

55

giving off oxygen e. g. caesium-permanganate, is heated until the pressure gauge 14 indicates that the necessary quantity of oxygen has been generated for transforming the metallic caesium layer in the bulb 1 into a photo-electrically active alkali metal-oxide layer. For the exact determination of the quantity of oxygen generated, it is, of course, necessary to know the volume of the part 15, which may be shut-off from the device by closing the cocks 7, 8 and 12. After closing the cock 9 the oxygen passes into the bulb 1 by opening the cock 8. By cooling the reservoir 16 with liquid air residual vapors or gases, other than oxygen, are prevented from passing into the bulb 1. After oxidation the cock 8 is closed and the cock 9 is opened and the bulb 1 evacuated a second time. Then the reservoir 17 containing e. g. caesium, is heated, to vaporize the alkali metal therein which is deposited on

the caesium-oxide layer in the bulb 1. After a third evacuation the tube is separated from the pumping device, is sealed, and is now ready for use.

What I claim is:

A method of producing a photoelectric active layer in a photoelectric tube which consists of depositing a metal coating on the inner wall of the bulb of the tube, evacuating said bulb, depositing a coating of an alkali metal on said metal coating, introducing a predetermined amount of oxygen into said bulb just sufficient to convert said alkali metal coating into a photoelectric active oxide of the alkali metal, evacuating the bulb a second time and then depositing a coating of free alkali metal on said layer of alkali metal oxide.

PAUL GÖRLICH.